

## UNITED STATES PATENT OFFICE

2,188,124

NONHYGROSCOPIC MATCH AND PROCESS  
FOR PRODUCING SAMEAlbert Blaine Doran, Los Angeles, Calif., assignor  
to Herbert R. MacMillan, Los Angeles, Calif.No Drawing. Application July 24, 1937, Serial  
No. 155,521. Renewed October 23, 1939

4 Claims. (Cl. 52—25)

This invention relates to matches and has for its principal object the production of match heads and, in combination, match heads with friction surfaces for igniting, which are so compounded as to be highly water repelling, or non-hygroscopic.

As heretofore manufactured, match heads and friction surfaces for igniting the same are composed largely of water absorbing, or water soluble, materials of such hygroscopic character that contact with water renders the match and said friction surface useless even with limited immersion.

This is particularly true in localities where the relative humidity is high, so that humidity alone is frequently a cause of decomposition and deterioration.

It is therefore, an object of this invention to provide a match head and a friction igniting surface therefor which is highly resistant to the absorption of moisture.

The composition of materials used herein may include the usual compositions for matches heretofore known as to igniting and burning elements and substantially any of such known compositions may be used with the improvements herein set forth to render matches made from such well known compositions highly nonhygroscopic.

In general, match heads are compounded from a selection of—

(1) Igniters, such as metallic oxides, chromates, chlorates or nitrates. As illustrative of these, the most common and most preferably used are lead oxide ( $Pb_2O_3$ ) and ferrous oxide ( $FeO$ ).

(2) Protective agents for igniters, such as the oxalates of the alkaline earth metals (Ba, Ca, Sr), or the like.

(3) Binders to hold the ingredients together, such as glue, starch, dextrine or other water soluble adhesives.

(4) Coloring matter, such as dyestuffs, pigments, metallic oxides or sulphates, or the like.

(5) Bulk fillers for volume, such as starch, diatomaceous earth, finely ground silica, flue dust or the like.

(6) Hardeners, such as formaldehyde or other aldehydes which function to give a degree of hardness and also to limitedly inhibit moisture absorption.

In addition to the above, there are many variations and selections of other materials well known, all of which however do not vary greatly in their inability to repel moisture, and thus deterioration and decomposition of such compounds proceed rapidly in the presence of high humidity.

This invention has for a further object the

modification of match compositions by the inclusion of a resinous material comprising esters formed by the reaction of polybasic acids with polyhydric alcohols and by such inclusion a reduction of the above described ingredients is also 5 accomplished.

In compounding the novel match head of the invention, polybasic acids such as phthalic, succinic, maleic, adipic, diphenic, naphthalic, or other dicarboxylic or polybasic acids, may be reacted 10 with polyhydric alcohols such as glycerol, glycols, or other polyhydric alcohols to a point at which esterification will take place.

The degree of esterification may well only proceed to a point at which the resinous condensation product can be dissolved in an aromatic solvent such as benzol but the product may comprise a mixture of partially esterified and completely esterified alcohols which is soluble in aromatic hydrocarbons but insoluble in water and 20 which, due to adhesive binding, hardness, and relatively high melting point qualities makes the esterification product particularly adapted as a combined binder, protective agent, and hardener for match head compositions while giving 25 improved ignition scratch surfaces.

As merely illustrative of a method of preparation, dihydroxy acids, such as stearic acid, may be reacted with trihydroxy alcohols, such as glycerol, or phthalic anhydride reacted with glycerol. 30 Many combinations of polybasic acids with polyhydric alcohols will be apparent to those skilled in the art to obtain suitable esters for the herein described purpose.

For instance, a mixture of 144 parts by weight 35 of phthalic anhydride may be heated with 97 parts by weight of glycerol to about 200° C., or from about 175° C. to 225° C. sufficient to obtain the desired esterification.

At this point, 71 parts by weight of oleic acid 40 together with 70 parts by weight of castor oil are added and heating continued at 200° C. for about one hour until the esterified product can be dissolved in a mixture of 95% benzol and 5% turpentine in quantity sufficient to form a free 45 flowing solution.

To the above solution mixture are then added 20 parts by weight of finely ground glass, 10 parts by weight of sulphur, 30 parts by weight of potassium chlorate, and 12 parts by weight of lead 50 dioxide.

The mixture is then well agitated and aerated until its volume increases about 25% by suspension of air at which time it is in suitable condition for dipping in the match sticks to which the 55

composition adheres to be then placed in a suitable drying locality to evaporate the solvent and thus yield one form of the subject of this invention.

Coal tar aromatics, hydrogenated petroleum solvents, lacquer and paint diluents, and other solvents may be used.

The action of the fatty oils, such as oleic acid, soy bean oil, castor oil, the fatty acids derived from linseed oil, walnut oil, or raw tung oil, or other similar fatty oils is effective to modify the condition of the esterification products to produce a relatively quick drying match head having the desired hardness and other qualities. As compared with known match heads, which require several hours drying time as a rule under the same conditions, the esters of the present invention by modification with the proper oils will dry in well under a second with proper working conditions.

I claim:

1. A composition for matches including: an igniting element, a bulk filler, and a combined hardener and binder therefor consisting of a polyhydric alcohol esterified with a polybasic acid.
2. A composition for matches including: an igniting element, a bulk filler, and a combined

hardener and binder therefor consisting of a polyhydric alcohol esterified with a polybasic acid and modified with a fatty oil; said composition being soluble in a hydrocarbon solvent and insoluble in water.

3. The process of preparing water resistant match heads, which comprises: esterifying a polyhydric alcohol with a polybasic acid at a temperature between about 175° C. and 225° C., continuing the heating at about the same temperature in the presence of added fatty oil until the resulting product when cooled is soluble in an added hydrocarbon solvent, mixing with the solution thus produced ignition and filling material, then evaporating the solvent.

4. The process of preparing water resistant match heads, which comprises: esterifying a polyhydric alcohol with a polybasic acid at a temperature between about 175° C. and 225° C., continuing the heating at about the same temperature in the presence of added fatty oil until the resulting product when cooled is soluble in an added hydrocarbon solvent, mixing with the solution thus produced ignition and filling material, aerating the mixture, then evaporating the solvent.

ALBERT BLAINE DORAN.